# EUROPEAN PATENT SPECIFICATION

(11) **EP 0 138 410 B1**
(45) Date of publication and mention of the grant of the patent: **20.05.1987**
(21) Application number: 84306414.8
(22) Date of filing: 19.09.1984
(51) Int. Cl.: C11D 3/40

(54) **Process for the manufacture of coloured detergent powder**
Verfahren zur Herstellung von gefärbtem Detergenspulver
Procédé pour la manufacture d'une poudre de détergent colorée

(30) Priority: 21.09.1983 GB 8325326
(43) Date of publication of application: 24.04.1985
(73) Proprietor: UNILEVER PLC, London EC4P 4BQ (GB); UNILEVER N.V., 3013 AL Rotterdam (NL)
(72) Inventor: Davies, Richard Llewellyn, Wirral Merseyside (GB); Don, Nigel Anderson, Bebington Merseyside L63 9HJ (GB)
(74) Representative: Mole, Peter Geoffrey

## Description

This invention relates to a process for the manufacture of uniformly coloured detergent powder.

Coloured detergent powders are normally made by adding dye or pigment to a crutcher slurry and converting the slurry to a powder by spray-drying. Alternatively dye solution can be injected into the main feed to the nozzles of the spray-drying tower with similar results. The disadvantage of these processes is that they contaminate the whole of the spray-drying plant with colour so that when a white powder is subsequently to be made it is necessary to clean down, with consequent loss of production time.

One of the ways of avoiding this disadvantage is to spray a solution of dyestuff onto white powder. The main difficulty with this is that of contacting each individual particle, to an equal extent. If that is not achieved, then a speckled or mottled powder results.

United States Patent No. 4 162 228 relates to a method of colouring detergent flakes which contain nonionic surfactant as an essential component. The method involves mixing a dry colourant into the flakes whereupon the nonionic surfactant dissolves the colourant, imparting an overall hue to the flakes. Flakes are, of course, easier to colour than powder since they are translucent, and the whole formulation is contained within the flake. In contrast, powders normally consist of two components - a spray-dried portion and a dry-dosed portion which may have different affinities for colourant resulting in the powder having a mottled appearance.

GB-A-1375108 (Procter & Gamble) discloses a process for manufacturing a granular detergent composition containing a water-soluble blue dyestuff such as Polar Brilliant Blue or Ultramarine Blue yet which is substantially uncoloured in the dry state. The composition is prepared by mixing the dyestuff in dry form with a detergent powder or a granular ingredient thereof, and then spraying it with a liquid agglomerating agent.

These prior art processes involving the mixing of a dry colourant with a powder or flake detergent composition or ingredient thereof have led to products which are either non-uniformly coloured or not coloured at all.

We have now discovered contrary to what would have been expected that uniformly coloured powder can be manufactured by simply mixing a particulate colourant with a detergent powder, if the particulate colourant comprises both a pigment (water-insoluble) and a dyestuff (water-soluble).

Accordingly, the present invention, provides a process for the manufacture of a uniformly coloured detergent powder which comprises admixing with a detergent powder a particulate colourant comprising a water-insoluble pigment and a water-soluble dyestuff.

If desirable or necessary, after the mixing step the coloured powder may be sprayed with a small percentage, for example 1-5% by weight, of water or of an ethoxylated alcohol nonionic surfactant in liquid or molten form. This can help to accentuate the colouration.

When choosing the colourant system it is important to select substances which will colour the powder adequately and yet not produce staining problems in the wash. We have found a combination of the pigment Ultramarine Blue, the dyestuff Duasyn^{O} Acid Blue and the blue-whitener Polar Brilliant Blue to give excellent results on all types of detergent powder.

Other dyestuffs which have been found to be satisfactory are Carbolan^{@}Violet, Gulf Acid Blue 6JS0 and Milling Blue 2BR, all of which are available from Imperial Chemical Industries Limited.

Preferably the mean particle size of the colourant is 0.5 to 5 pm, most preferably about 2 um.

The process may be applied to powder which has been prepared by spray-drying, spray-cooling, granulation or agglomeration or any combination of these techniques. Additionally, any of the powder so produced may be dosed with conventional detergent powder additives such as sodium perborate tetrahydrate without altering the effectiveness of the process.

The apparatus used for mixing the particulate colourant and the powder is not critical to the process. We have found a rotating drum mixer to be perfectly satisfactory and also, a Patterson-Kelley (Registered Trade mark) batch blender has performed well.

The invention will be further described in the following example.

### Example

White, spray-dried detergent powder is first fed down a chute at a flow rate of about 350 Kg/hdur controlled by a slide valve into one end of the interior of a rotatable drum mixer without internal baffles. The axis of the drum mixer is approximately horizontal but the mean residence time of the powder in the drum which is about 2 minutes can be adjusted to some extent by moving the axis up or down by a few degrees. The drum is rotated and a finely powdered mixture of the following colourants is fed into the drum from a variable speed dosing unit:

Substantially uniformly blue coloured powder emerges from the discharge end of the drum mixer.

If desired the small quantity of water or nonionic surfactant referred to above, say 1-3% by weight may be sprayed onto the powder in the drum through spray nozzles located along the axis.

There are several advantages to the process described above. Most importantly it avoids colouration of the spray-drying plant, but also it appears to be independent of formulation, and is suitable for colouring fully-formulated powder and not just the spray-dried portion.

## Claims

1. A process for the manufacture of a uniformly coloured detergent powder, characterised in that there is admixed with a detergent powder a particulate colourant comprising a water-insoluble pigment and a water-soluble dyestuff.

2. A process as claimed in claim 1, characterised in that the particulate colourant comprises the blue pigment Ultramarine Blue and a dyestuff selected from Duasyn^{O} Acid Blue, Carbolan- ^{®}Violet, Gulf Acid Blue 6 JSO and Milling Blue 2BR.

3. A process according to claim 1 or claim 2, characterised in that the coloured powder is sprayed with from 1 to 5% by weight of water.

4. A process according to claim 1 or claim 2, characterised in that the coloured powder is sprayed with from 1 to 5% by weight of an ethoxylated alcohol nonionic surfactant in liquid or molten form.

5. A process according to any one of the preceding claims characterised in that the mean particle size of the colourant is from 0.5 to 5 µm.

6. A process according to claim 5, characterised in that the mean particle size of the colourant is about 2 µm.

## Patentansprüche

1. Verfahren zur Herstellung eines einheitlich gefärbten Detergenspulvers, dadurch gekennzeichnet, daß zu einem Detergenspulver ein teilchenförmiges Färbemittel, das ein wasserunlösliches Pigment und einen wasserlöslichen Farbstoff umfaßt, zugemischt wird.

2. Verfahren nach Anspruch 1, dadurch gekennzeichnet, daß das teilchenförmige Färbemittel das blaue Pigment Ultra-marinblau und einen Farbstoff ausgewählt unter Duasyn⁸ Acid Blue, Carbolan^{@} Violet, Gulf Acid Blue 6 JSO und Milling Blue 2BR umfaßt.

3. Verfahren nach Anspruch 1 oder 2, dadurch gekennzeichnet, daß das gefärbte Pulver mit 1 bis 5 Gew.-% Wasser besprüht wird.

4. Verfahren nach Anspruch 1 oder 2, dadurch gekennzeichnet, daß das gefärbte Pulver besprüht wird mit 1 bis 5 Gew.-% eines ethoxylierten Alkohol-nonionic-Tesids in flüssiger oder geschmolzener Form.

5. Verfahren nach einem der vorhergehenden Ansprüche, dadurch gekennzeichnet, daß die mittlere Partikelgröße des Färbemittels von 0,5 bis 5 um beträgt.

6. Verfahren nach Anspruch 5, dadurch gekennzeichnet, daß die mittlere Partikelgröße des Färbemittels etwa 2 µm beträgt.

## Revendications

1. Procédé de fabrication d'une poudre détergente uniformément colorée, caractérisé en ce qu'on mélange avec une poudre détergente un colorant particulaire comprenant un pigment insoluble dans l'eau et un colorant soluble dans l'eau.

2. Procédé selon la revendication 1, caractérisé en ce que le colorant particulaire comprend le pigment bleu Bleu Outremer et un colorant choisi parmi le Bleu Acide Duasyn (marque déposée), le Violet Carbolan (marque déposée), le Bleu Acide Gulf 6 JSO et le Bleu de Broyage 2BR.

3. Procédé selon la revendication 1 ou 2, caractérisé en ce qu'on pulvérise sur la poudre colorée de 1 à 5% en poids d'eau.

4. Procédé selon la revendication 1 ou 2, caractérisé en ce qu'on pulvérise sur la poudre colorée de 1 à 5% en poids d'un surfactif non ionique à base d'alcool éthoxylé sous forme liquide ou fondue.

5. Procédé selon l'une quelconque des revendications précédentes, caractérisé en ce que la granulométrie moyenne du colorant est de 0,5 a 5 µm.

6. Procédé selon la revendication 5, caractérisé en ce que la grosseur moyenne des particules du colorant est d'environ 2 ^{p}m.
